

## UNITED STATES PATENT OFFICE.

OSCAR LINDER, OF CHICAGO, ILLINOIS, ASSIGNOR TO IDEAL ROLLER AND MANUFACTURING CO., OF CHICAGO, ILLINOIS, A CORPORATION OF ILLINOIS.

## PROCESS FOR MOLDING ARTICLES.

No Drawing.

Application filed November 17, 1919. Serial No. 338,419.

This invention relates to a new process for molding articles and more particularly to the molding of articles which are made of vulcanized oils such as rollers, platens, 5 tire-filers, etc.

It is well known to those skilled in the art that many oils, particularly oils of vegetable origin, such as corn oil, cotton seed oil, linseed oil, rapeseed oil, and soya-bean oil, and 10 also other oils, such as fish oils, etc., can be hardened or solidified by vulcanizing them with sulphurchloride, sulphur or other similar vulcanizing agents which will convert such oils into a resilient and plastic mass 15 which is somewhat similar to rubber.

A very extensive use of this process is made, for example, in the production of printers' and lithographers' rollers, in which process the particular oil used is generally 20 mixed at atmospheric or room temperature with from 10% to 40% of its weight of sulphurchloride, after which the resulting liquid mixture is poured into a suitable mold where it hardens within a few minutes by 25 virtue of the chemical action resulting between the two ingredients into a solid but soft and resilient mass, after which it can be removed from the mold.

The process of making molded vulcanized 30 oil articles, as heretofore practiced, had the great disadvantage in that the resulting mass generally contained gas cells of minute size which rendered the mass somewhat porous and correspondingly ununiform and weak, 35 and which also resulted in an uneven surface. Many expedients have been resorted to for the purpose of overcoming this objectionable feature in the vulcanization process, but with no apparent success. The 40 gas cells which occur in the mass are due largely to liberation of acid gases such as hydrochloric acid and sulphur dioxide during the chemical reaction and at the time when the mass is in the process of hardening, 45 so that these gas cells have no opportunity to escape before the mass has hardened.

According to the new process herein described, these gas cells referred to can be 50 eliminated, or, if not entirely eliminated, at least reduced to such a minute size that their presence cannot be readily detected. The 55 improved process consists essentially in subjecting the mass to pressure after it has been poured into the mold at atmospheric or room temperature and while it is undergoing

the process of vulcanization. The mass can be subjected to pressure in a large variety of ways. Thus, for example, by placing the mold, which contains the liquid mixture of oil and sulphurchloride in a closed receptacle and then subjecting the mass contained in the mold, positioned in the receptacle, to an air pressure of suitable magnitude until the chemical reaction is completed and the mass has hardened as desired. The air pressure is then relieved, the mold removed from the receptacle, and the molded article removed from the mold. Obviously any other desired method of applying the pressure to the mass could be readily utilized by those 70 skilled in the art.

The application of this external pressure to the mass in the mold serves to effectively prevent the liberation of free gases at least as far as can be determined by optical 75 means; for example, with the help of a microscope and by physical tests, as for example, by the determination of the density of the mass. If there are any gas cells in the resulting mass prepared in accordance with 80 the teachings of this invention, they, therefore, must be of such minute size that they cannot be readily detected. The resulting hardened or vulcanized oil, produced according to this process in molded form is much 85 more uniform, stronger, and has a much smoother surface than a corresponding article made without the aid of pressure. The new process as herein described is, therefore, adapted to be used for the ready molding 90 of articles which can and could not heretofore be molded satisfactorily by the old process on account of the porosity and the rough surface of the resulting article.

In the place of vulcanization, the oils 95 may be hardened by other processes such as oxidation, hydrogenation, polymerization, etc., with each of which obviously some means of applying pressure to the mass during the period of vulcanization is utilized, 100 if the resulting molded body is to be uniformly solid and resilient and free from apparent porosity or gas and air cells.

For the purpose of preventing the adhesion of the solid mass to the mold and 105 to provide for the ready removal of the molded mass from the mold, the mold is preferably coated with some inert material such as paraffin, vaseline, glycerine, soap or the like. Obviously, the pressure can be 110

produced in any desired manner but is preferably obtained by the use of compressed air. The pressure obviously may be of any desired amount, so long as it exceeds the atmospheric pressure, but ordinarily and for general purposes a pressure of about 50 pounds per square inch is found to be the most desirable. The pressure may obviously be applied at any time after the unhardened mass has been poured into the mold and before the vulcanization or hardening has taken place, and said pressure must be kept on continuously until the vulcanization is completed. As soon as the chemical reaction is completed the pressure can be released, after which the hardened mass may be removed from the mold.

Although the oils referred to hereinbefore are mainly and preferably used with the new process herein described, the process is obviously not restricted specifically to the oils enumerated but may be used with any oil which can be hardened or vulcanized, or any other substance which is liquid at ordinary temperatures and which can be hardened through vulcanization. Likewise, mixtures of various oils may be used or compounds of oils and varnishes, or any other combinations which can be readily poured in liquid state at ordinary temperatures. Likewise, in the cold vulcanization process, instead of using pure or concentrated sulphur chloride, a sulphur chloride diluted with any diluent, such as benzol, carbon bisulphide, etc., may be used. Ob-

viously, likewise, any suitable or desirable mixtures of the oil may also be used. While the so-called "cold" vulcanization takes place without the application of heat, there is a very slight raise in the temperature due to the chemical reaction.

The invention is obviously not limited to the specific embodiments thereof herein described, but is capable of many variations and other applications within the scope and spirit thereof as set out in the following claims:

Having thus described my invention, what I claim as new and desire to secure by Letters Patent is:

1. The process of molding resilient articles which consists in vulcanizing fatty oils at room temperature under pressure for the purpose of retaining the greater portion of the air and gas cells in the article and reducing the size thereof sufficiently so that they will not be detrimental to the finished product.

2. The process of molding resilient articles which consists in vulcanizing oils at room temperature with sulphur chloride under pressure for the purpose of retaining the greater portion of the air and gas cells in the article and reducing the size thereof sufficiently so that they will not be detrimental to the finished product.

In witness whereof, I have hereunto subscribed my name.

OSCAR LINDER.